# EUROPEAN PATENT SPECIFICATION

(11) **EP 3 821 041 B1**
(45) Date of publication and mention of the grant of the patent: **08.10.2025**
(21) Application number: 19741994.8
(22) Date of filing: 11.07.2019
(51) Int. Cl.: C21D 6/00, C21D 8/02, C21D 1/18, C21D 1/25, C22C 38/00, C22C 38/04, C22C 38/06, C22C 38/14, C22C 38/60

(54) **PROCESS FOR PRODUCING A HIGH STRENGTH COLD-ROLLED AND HEAT-TREATED STEEL STRIP AND PRODUCT PRODUCED THEREBY**
VERFAHREN ZUR HERSTELLUNG EINES HOCHFESTES KALTGEWALZTEN UND WÄRMEBEHANDELTEN STAHLBANDS UND DADURCH HERGESTELLTES PRODUKT
PROCÉDÉ DE PRODUCTION D'UNE BANDE D'ACIER LAMINÉE À FROID À HAUTE RÉSISTANCE ET TRAITÉE THERMIQUEMENT ET PRODUIT AINSI OBTENU

(30) Priority: 11.07.2018 EP 18182906
(43) Date of publication of application: 19.05.2021
(73) Proprietor: Tata Steel Nederland Technology B.V., 1951 JZ Velsen-Noord (NL)
(72) Inventor: CHEN, Shangping, 1970 CA IJmuiden (NL); XIAO, Bin, 1970 CA IJmuiden (NL); MOSTERT, Richard, 1970 CA IJmuiden (NL)
(74) Representative: Group Intellectual Property Services
(86) International application number: PCT/EP2019/068659
(87) International publication number: WO 2020/011911

(56) References cited:
- EP-A1- 3 088 546
- EP-A1- 3 421 629
- US-A1- 2016 017 469
- US-A1- 2016 312 323
- US-A1- 2017 327 919
- LEE SEONJONG ET AL: "Tensile Properties of Medium Mn Steel with a Bimodal UFG [alpha] + [gamma] and Coarse [delta]-Ferrite Microstructure", METALLURGICAL AND MATERIALS TRANSACTIONS A: PHYSICAL METALLURGY & MATERIALS SCIENCE, ASM INTERNATIONAL, MATERIALS PARK, OH, US, vol. 48, no. 4, 7 February 2017 (2017-02-07), pages 1678 - 1700, XP036185841, ISSN: 1073-5623, [retrieved on 20170207], DOI: 10.1007/S11661-017-3979-Z
- CHOI HONGKI ET AL: "Characterization of fracture in medium Mn steel", MATERIALS SCIENCE AND ENGINEERING: A, ELSEVIER, AMSTERDAM, NL, vol. 687, 21 January 2017 (2017-01-21), pages 200 - 210, XP029919170, ISSN: 0921-5093, DOI: 10.1016/J.MSEA.2017.01.055
- SOHN S S ET AL: "Effect of annealing temperature on microstructural modification and tensile properties in 0.35 C-3.5 Mn-5.8 Al lightweig", ACTA MATERIALIA, ELSEVIER, OXFORD, GB, vol. 61, no. 13, 25 May 2013 (2013-05-25), pages 5050 - 5066, XP028572549, ISSN: 1359-6454, DOI: 10.1016/J.ACTAMAT.2013.04.038

## Description

This invention relates to a high strength cold-rolled and heat-treated steel strip and strip produced thereby, useful for producing frame components for vehicles and automobiles such as frames for trucks.

In recent years, (advanced) high strength steel sheets, AHSS, are increasingly used in car components to reduce weight and fuel consumption. A series of (advanced) high strength steels, such as HSLA, Dual phase (DP), Ferritic-bainitic (FB) including stretch-flangeable (SF), Complex phase (CP), Transformation-induced plasticity (TRIP), Hot-formed, Twinning-induced plasticity (TWIP) has been developed to meet the growing requirements.

However, AHSS sheet steels cannot be applied easily to a wide variety of car components because their formability is relatively poor. As steels became increasingly stronger, they simultaneously became increasingly difficult to form into automotive parts. Actually, the application of AHSS steels (DP, CP and TRIP) to car components is still limited by their formability. Therefore, improving formability and manufacturability is an important issue for AHSS applications.

To achieve a high yield strength/tensile strength ratio and an even higher tensile strength, i.e. above 800 MPa, steels having complex microstructures (ferrite, bainite martensite and/or retained austenite) have been developed.

Transformation-induced plasticity (TRIP) steel is one of these high-strength steels that utilize phase transformation to control the mechanical properties. Strain-induced martensitic transformation of metastable austenite plays a major role in improving the mechanical balance (tensile strength x elongation), allowing TRIP steel to be actively applied in the automotive industry. Currently, the tensile strength of commercially produced TRIP steel reaches approximately 1000 MPa. However, when the tensile strength exceeds 800 MPa, the elongation tends to decrease to less than 15 % and the mechanical balance is significantly deteriorated. A microstructural control ensuring higher stability as well as a sufficient fraction of retained austenite would be essential to obtain a higher tensile strength with desirable elongation.

Low-carbon, manganese TRIP steel (Mn TRIP steel) based on an alloy system of Fe-0.1C-5Mn was first introduced by Miller [R.L. Miller: Metall. Trans., 1972, vol. 3, pp. 905-12]. A retained austenite fraction of 20 ~ 40 % with optimized stability made it possible to exhibit an excellent mechanical balance after intercritical annealing. However, a prolonged heat treatment using a batch-type annealing process was required to obtain the desired properties.

Grain refinement of steels to submicron size and nano size has also been used to explore the improvement of the strength of metals. However, it has been reported that the ductility of ultra-fine grained (UFG) metals decreases as the grain size is reduced below 5 µm. The uniform elongation turns to almost zero when grain size becomes less than 2 µm. For the UFG materials, fracture occurs immediately after yielding during plastic deformation at room temperature. The low ductility in ultrafine-grained metals and alloys is attributed to their very poor work hardening capacity caused by their inability to accumulate dislocations because of their small grain size and saturation of dislocations, which seems to be a size effect intrinsic to small plastic domains. This indicates that it is difficult to manufacture products such as vehicle and aircraft components made of ultrafine-grained metals, particularly nano-crystalline metals, through secondary plastic deformation methods such as forging, pressing, and drawing. SOHN S.S. et al. in "Effect of annealing temperature on microstructural modification and tensile properties in 0.35C - 3.5Mn - 5.8Al lightweight steel", Acta Mat., no. 13/2013, p. 5050/66 and EP3421629-A1 describe manufacture of similar steels.

It is an object of the present invention to provide a process for producing a steel grade which combines a high strength with a good elongation.

It is also an object of the present invention to provide a steel grade which combines a high strength with a good elongation.

The invention is defined in the appended claims.

According to a first aspect one or more of the objects of the invention may be reached with a process for producing a high strength cold-rolled and heat-treated steel strip, sheet, blank or hot-press-formed product having a bimodal microstructure comprising the steps of claim 1.

In an embodiment the sum of the α-ferrite, bainite, martensite and retained austenite is between 10 and 90 vol. %.

A cooling rate CR2 of higher than 10 °C/s is usually sufficient to prevent the decomposition of the austenite for the compositions of the steel according to the invention. A suitable maximum cooling rate is 100 °C/s, preferably at most 75 °C/s, more preferably 50 °C/s. The cooling rate (CR3) after the optional austempering treatment is preferably from 0.01 °C/s to 50 °C/s. If the duration of maintenance at the austempering temperature is 0s, then there is no austempering.

Ambient temperature is defined as the temperature of the surrounding air, and is also referred to as room temperature. The Oxford English Dictionary defines a typical value for room temperature to be 20 °C.

The bimodal grain size distribution is essential in these steels. With the bimodal size distribution of grains in the microstructure, the restricted ductility of UFG steels due to the high strain-hardening capacity of the coarse grains and strengthening ability of the ultrafine grains can be overcome and provides a good combination between strength and elongation.

This invention is to provide steels with a high strength and a high formability. The invented steel sheets are multi-phase steels including δ-ferrite, α-ferrite, martensite and/or bainite and retained austenite and having a bimodal microstructure, in which the δ-ferrite has a relative large grain size range from 5-20 µm, while the α-ferrite and other phases have a small grain size < 5 µm.

The steel consists of δ and α ferrite, and the minimum amount of Σ(δ+α) is at least 30 vol.%. The sum of the bainite, martensite and retained austenite phases is between 10 and 70 vol.%. Consequently, the maximum amount of Σ(δ+α) is 90 vol.%. A suitable maximum for the δ-ferrite is 80 vol%, preferably 70 vol.%, more preferably 60 vol.%.

Figure 1 gives a schematic indication of the phases in pure iron during slow cooling from the liquid phase (L). As pure iron cools, it changes from one phase to another at constant temperatures. Pure iron solidifies from the liquid at 1538 °C (top of Fig. 1). A crystalline body-centred cubic lattice (bcc) structure, known as δ-ferrite, is formed (point a). As cooling proceeds further and point b (Fig. 1) is reached (1395 °C), the atoms rearrange into the face-centred cubic lattice (fcc), and this structure is called γ-iron or austenite. As cooling further proceeds to 910 °C (point c), the structure reverts to the bcc structure and this low temperature bcc-phase is called α-ferrite. The change at point d (770 °C) merely denotes a change from paramagnetic to ferromagnetic iron and does not represent a phase change (the magnetic transformation is usually considered to be a second order phase transformation, and the temperature at which this occurs is the Curie-temperature). The entire field below 910 °C is composed of α-ferrite, which continues down to room temperature and below. This principle applies also to iron-based alloys, although the transformation temperatures are strongly influenced by the alloying additions to the iron. These influences can be made visible with the so-called phase diagrams.

So, the δ-ferrite is a ferritic phase originating from the solidified steel and the likelihood of its forming is increased as a result of the selected composition. Also, whether or not it remains stable at ambient temperature depends on the composition as well. The required amount of the δ-ferrite in the final microstructure of the steels according to the invention is at least 10 % in volume.

C is a necessary element for strength and hardenability.

The austenite phase is enriched with C on annealing in the α-γ intercritical region as well as during austempering of a bainitic structure. The higher carbon content in the austenite contributes to lowering the Mₛ, martensite start transformation temperature. The C enriched in the austenite stabilises the austenite to form residual austenite at ambient temperature. Upon deforming some amount of the residual austenite transforms to martensite and thus contributes to the strength after deformation, whilst being relatively ductile before deformation. Thus, it is required that the C content is controlled at an appropriate level so as to control the desired microstructure and maintain the delicate balance of microstructure and properties. For the steels according to the invention the carbon content is from 0.05 to 0.50 wt.% (all compositional percentages are in weight percent (wt.%) unless otherwise indicated). A suitable minimum amount is 0.080 %, preferably at least 0.10 %. A suitable maximum amount is 0.46 %, more preferably at most 0.40 %.

Silicon and aluminium are ferrite forming elements which are added to promote the formation of the δ-ferrite in the microstructure. These elements also increase the concentration of C in austenite and suppress the formation of carbides and thus have the function to promote the formation of residual austenite. The sum total of Si and Al is from 0.10 to 6.50 %. Silicon is preferably between 0.050 % and 2.00 %, the upper boundary being dictated by steel surface quality. Aluminium is preferably between 0.050 and 6.00 %. A high content of Al results in a steel sheet exhibiting a high value in a total elongation while maintaining a high strength. However, if Al is excessively added, x-carbide may be formed during intercritical annealing and a disorder (bcc_A2) to order (bcc_B2) transition will occur in the ferrite at a lower temperature. The presence of κ-carbide in the microstructure is undesired, and its formation should be prevented. Preferably the microstructure of the high strength cold-rolled and heat-treated steel is free from κ-carbide. The formation of the ordered structure reduces the ductility of steel, so that the upper limit of aluminium is restricted to 6 %. A suitable minimum amount of aluminium is 0.75 %. In a preferable embodiment the minimum amount of aluminium is 1.50 %, or even 2.50 %. Preferably the sum total of Si and Al is at least 2.50, preferably at least 2.75, more preferably at least 3.00 %. Preferably the aluminium content is at most 5.50 wt.%, more preferably at most 5.00 wt.%, even more preferably at most 4.80 wt.% or even at most 4.70 wt.%.

The amount of Si and Al needs to be adjusted according to the total amount of Σ(Mn+Cu+Ni) to guarantee the presence of the δ-ferrite and complete recrystallization in the δ-ferrite during annealing at the intercritical (γ + δ) temperatures. To ensure the formation of δ-ferrite, the following equation has to be satisfied (in wt.%): $Al + \left(Si/3\right) \geq 4 \times C + 0.24 \times \sum \left(Mn+Cu+Ni\right) + 0.9$

The functions of manganese are to stabilize the austenite and to harden the steel. Below 0.50 % these effects are not sufficiently marked. If the content of Mn increases, the phase transformation points A₃ and A₁, the martensite and the bainite transformation temperatures are lowered. The recrystallization temperature of the ferrite phase is increased and recrystallization kinetics of ferrite is decreased. Higher amounts of ferritic stabilizers, such as Al and Si are needed to increase the (δ + γ) phase field to guarantee the formation of the δ-ferrite. Thus, the level of Mn is limited to at most 8.00 %, and preferably to at most 7.00 %, and even more preferably at most 6.00 %.

Cu and Ni can optionally be used at amounts of up to 2.00 % Cu and 2.00 % Ni to partly replace Mn, but the total amount of Cu, Mn and Ni must be in the range of 0.50 to 8.00 %, preferably to at most 6.50 %. The added copper may provide precipitation hardening. Moreover, because the copper is insoluble in the cementite, it has a beneficial effect on the residual austenite, similar to silicon and aluminium. Preferably copper is at most 0.15 wt.%

Sb is an important element for steels containing high amounts of alloying elements such as Al, Mn and Si. Sb itself does not form an oxide thin film at high temperatures but is enriched into the surface and the grain boundaries. As a result, Sb inhibits Al, Mn and Si from diffusing to the surface, which results in inhibiting the oxidation of these elements. Thus, the addition of minute amounts of Sb has an unexpected and remarkable effect on the occurrence of MnO, SiO₂, Al₂O₃, etc. during annealing a cold-rolled steel sheet. In order to produce these effects only small amounts of Sb are required, and 0.0005 % (5 ppm) Sb already has an effect. So a preferable minimum amount is 0.0005 % Sb, more preferably at least 0.0010 % (10 ppm). If Sb is added beyond a specified limit, it brings grain boundary embrittlement. Thus, the content of Sb is limited to the upper limit 0.050 %, preferably to the upper limit of 0.0150 %, even more preferably 0.0100 % (100 ppm).

P is an impurity in the steel. P segregates at the grain boundaries and decreases the workability. Therefore, the amount of P should be suppressed to 0.050 % or smaller, preferably 0.010 % or smaller.

S is a harmful element which forms sulphide-based inclusions such as MnS, which may serve as a crack initiator, thereby deteriorating processability. Therefore, it is desirable to reduce the amount of S as much as possible. Accordingly, S is 0.020 % or smaller. Preferably S is 0.010 % or even 0.008 % or smaller.

Nitrogen (N) is inevitably present in the steel making process and allowable in the steels according to the invention in amounts between 5 to 100 ppm. The N content is preferably 60 ppm or less. Desirably, the N content is decreased as much as possible. A suitable and practical minimum N content is 10 to 50 ppm.

Boron (B) is a potent hardenability enhancer in low C, low alloy steels. B is a very effective alloying element in increasing the yield strength. The B content should preferably be at most 25 ppm so as not to impair low temperature toughness. For the boron to be able to perform this role, it is essential that no free nitrogen is present so that the formation of BN is avoided. This is where the nitrogen scavenging effect of certain elements such as titanium or aluminium comes in. A suitable minimum amount of Boron is 5 ppm.

At least one element selected from Ca: 0.0050 % or smaller and REM: 0.0050 % or smaller is used. These Ca and REM (rare earth element) are elements effective for controlling a form of sulphide in the steel and improving processability. Examples of the rare earth element include Scandium, Yttrium, and lanthanide. It is recommended that for these elements to be useful they have to be present in amounts of 0.0005 % or higher. However, when added excessively, the effect is saturated and the economic efficiency is reduced. Therefore, it is better to suppress an amount thereof to 0.0050 % or smaller, preferably to 0.0030 % or smaller.

Ti can also be added in a total amount preferably not exceeding 0.10 %. Ti forms carbides, nitrides or carbonitrides which block grain growth at high temperature and increase strength by precipitation. Preferably Ti does not exceed 0.050 %. If added, a suitable minimum amount is 0.0040 %

It is desirable to avoid the addition of elements which slow down the bainitic transformation. This applies for instance to Cr, Mo and V. In any event, the contents of each of these elements individually must preferably not exceed 1.00 %. Preferably, their total concentration (Σ(Cr+Mo+V)) must not exceed 0.30 %.

The other elements present in the steel are those usually found as manufacturing impurities, in proportions which have no significant effect on the required properties of steel. These residual elements (aka inevitable impurities, such as Cu, Ni, As, Pb, Sn, Mo, Cr, etc.) are defined as elements which are not added on purpose to steel and which cannot be removed by simple metallurgical processes. Some of the elements can be present as residual element, like nickel, but nickel can also be added to the steel during steelmaking, in which case it would no longer be a residual element or inevitable impurity, but an alloying element. In many cases it cannot be determined in the finished steel product whether (e.g.) nickel was added as an alloying element, or whether it was present as a residual element. Residual elements enter steel from impurities in ore, coke, flux and scrap; from these, scrap is considered to be the main source of residuals. Consequently, the level of residual elements in the Electric Arc Furnace process route (100% scrap based) is significantly higher than in the Basic Oxygen Steelmaking process route. The most commonly found residuals are Cu, Ni, Cr, Mo, and Sn. The acceptance limits of these residuals depend mainly on product requirements. Preferably the steel according to the invention is produced in a BOS-process route, in which case the allowable levels of residual elements for Cu, Ni, Cr, Mo and Sn are 0.040, 0.040, 0.040, 0.020 and 0.020 wt.% respectively.

The process according to the invention results in a heat-treated strip, a heat-treated sheet by using a continuous annealing line, or a heat-treated blank, a heat-treated product obtained by hot-press forming, or a product cold-formed from the blank and subsequently heat-treated. If the sheet or blank is heat treated according to the invention with the intention to hot-press-form the heat-treated sheet or blank into a hot-press-formed product, then it will be clear that the sheet or blank to be hot-press-formed is brought to the intercritical annealing temperature, preferably at a temperature between 600 and 900 °C, for a duration of between 1 and 600 s prior to hot-press-forming to attain the desired temperature and microstructure prior to forming, and that the hot-press-formed product is subsequently cooled to an austempering temperature for an austempering treatment between 500 and 300 °C, preferably at most 480 and/or at least 320 °C, at a cooling rate (CR2) which is higher than the critical rate for formation of pearlite, and maintained for a duration of 0 to 1200 s for austempering and subsequently cooled (CR3) to ambient temperature to obtain the desired bimodal grain microstructure, preferably at a cooling rate (CR3) of 0.01 °C/s to 50 °C/s. If the duration of maintenance at the austempering temperature is 0s, then there is no austempering.

In this embodiment wherein the blank (or sheet) undergoes the heat treating in a reheating furnace for a hot-forming press, wherein the intercritical annealing of the blank takes place before hot-press-forming in the hot-forming press, and the intercritically annealed blank (or sheet) is hot-pressed and cooled to the austempering temperature of between 500 and 300 °C, preferably at most 480 and/or at least 320 °C, in the hot-press and i). held in the hot-press for the duration of the austempering treatment or ii). taken from the hot-press and entered into an austempering furnace for the duration of the austempering treatment, followed by cooling to ambient temperature, preferably at a cooling rate (CR3) of 0.01 °C/s to 50 °C/s.

This is an example of the direct hot-forming process wherein the unformed blank (or sheet) is heated in a furnace, formed in hot condition, and quenched in the die to achieve the required temperature and thus microstructure and thus properties after which it is cooled in the press to ambient temperature, or taken out and cooled in an austempering furnace to ambient temperature.

In an embodiment the blank produced from the cold-rolled strip is first deformed in a press to form a product and the formed product subsequently undergoes the heat treating in an annealing furnace wherein the intercritical annealing of the product takes place and wherein
i) the intercritically annealed product is cooled to the austempering temperature of between 500 and 300 °C, preferably at most 480 and/or at least 320 °C, in the annealing furnace and held for the duration of the austempering treatment for 0 to 1200 s, followed by cooling to ambient temperature, preferably at a cooling rate of 0.01 °C/s to 50 °C/s, or
ii) wherein the intercritically annealed product is taken from the annealing furnace and entered into an austempering furnace at the austempering temperature of between 500 and 300 ° C, preferably at most 480 and/or at least 320 °C, followed by cooling to ambient temperature, preferably at a cooling rate of 0.01 °C/s to 50 °C/s.

This process is known as an indirect hot process: the blank is formed, trimmed, and pressed in cold condition. It is later intercritically annealed and cooled according to the invention to get high strength properties and the desired bimodal grain structure.

In an embodiment the duration of the intercritical annealing is at least 30 s and/or at most 400 s. The duration must be sufficiently long to obtain the right starting microstructure and not too long to cause problems with process control, undesirable grain growth or excessive energy consumption. The optimum time can be easily determined on the basis of simple experimentation. The same applies to the temperature and the duration of the austempering annealing which is preferably at least 30 s and/or at most 600 s. The austempering temperature is preferably at least 320 °C and more preferably at least 350 °C and/or at most 475 °C, and even more preferably at most 450 °C.

In an embodiment i) Σ(Mn+Cu+Ni) is between 0.50 and 8.00 wt.%, and/or ii) Σ(Al+Si) is between 0.10 and 6.50 wt.%, and/or iii) Al+(Si/3)≥24C+ Σ(Mn+Cu+Ni)+0.9. These three conditions i, ii, and iii are therefore combinable, meaning that the following combinations are possible: i, ii, iii, i+ii, i+iii, ii+iii, i+ii+iii.

Figure 2 shows the phase diagram of Fe-5.8Mn-3.2Al-0.25Si-xC steels as an example according to the current invention.

In the process according to the present invention a steel melt, preferably produced via a BOS-process route, is conventionally cast in the form of a thick slab, a thin slab or a strip. After casting it is brought to hot-rolling temperatures by (re-)heating and/or homogenising and hot-rolled, depending on whether the cast was made as a thick slab, a thin slab or a strip. The slab reheating temperature (SRT) or homogenisation temperature has to be sufficiently high to dissolve coarse Ti and V carbides which may have precipitated in the slab during casting or to keep them in solution in case of a thin slab casting and direct-rolling process. The inventors found that a SRT of at between 1100 and 1300 °C is preferable. A suitable maximum SRT is 1250 °C. The reheating of the slab or cast strip to the reheating temperature is a known process per se and the time needed to reheat the slab or strip to the reheating temperature depends inter alia on the type of furnace, the thermal capacity of the furnace, the thickness of the slab or strip. Typical residence times in a reheating furnace of a conventional hot strip mill are between 2 and 5 hours when starting from cold slabs. In a thin slab casting and direct rolling mill the slabs are not cooled but homogenised at the reheating temperature. Typical residence times in a reheating furnace of such a mill is typically between 5 and 120 minutes.

The hot-rolling pass is performed on the steels within the two-phase (γ + δ) field. So the microstructure during hot-rolling consists of γ-grains and δ-ferrite grains. During hot-rolling, recovery and/or recrystallization occur in the two phases. However, due to the difference in the recrystallization behaviour, the grains in the γ phase are refined through recrystallization, while the grains in the δ phase are coarser and present as elongated shape and the recrystallization is incomplete. On the other hand, partitioning of elements, C, Mn and Al occurs between the δ- and γ-phases and some amount of the α-ferrite forms within the γ phase as the hot rolling temperature gradually decreases. The microstructure at hot rolling finish temperatures consists of partially recrystallized bands of coarse grained δ-ferrite, bands of γ-austenite with smaller grains and small amount of α-ferrite within the γ bands. The hot-rolling finishing temperature is preferably between 800 °C to 950 °C. This temperature range is applied to produce fine grains in the austenite (y) and elongated laminate grains in the δ-ferrite.

The thickness of the hot-rolled strip according to the invention is between 1.5 and 10 mm. Preferably the thickness is at least 2 and/or at most 8 mm, more preferably at least 3 and/or at most 6 mm.

After finish rolling the steel is cooled on the run-out table of the hot strip mill, preferably at an average cooling rate of between 5 and 200 °C/s, more preferably of at least 10 and/or at most 150 °C/s, or even more preferably of at most 100 °C/s, to a coiling temperature of between 680 and 480 °C followed by cooling of the coil by natural cooling down to ambient temperature. During cooling and coiling, the γ phase decomposes into α-ferrite and carbides. If the cooling rate is too low or the coiling temperature is too high, carbides may form in a larger size along grain boundaries, which is detrimental to cold rolling. So the formation of coarse carbides must be avoided. The preferred average cooling rate ensures that the formation of coarse carbides is avoided.

The hot-rolled steel sheet is coiled at a temperature between 480 °C to 680 °C. In this temperature range, elements such as Si, Mn and Al in steel react with an oxide scale (FeO) after coiling, thereby forming alloyed oxides at a scale/metal interface. This formation of the Si, Mn and Al oxides has a strong influence on concentrations of these elements in the outermost surface layer of the strip. The addition of Sb has a suppressing effect on the formation of these alloyed oxides at very low additions.

If the coiling temperature is lower than 480 °C, undesirable amounts of low temperature transformation structures, such as bainite and martensite may be formed, which adversely affect the cold-rollability. When the coiling temperature exceeds 680 °C, then internal oxidation of Si, Mn and Al become problematic, and the inhibiting effect of Sb is no longer able to prevent this if the coiling temperature exceeds 680 °C. This has an adverse influence on surface roughness and pickleability. Preferably the coiling temperature is at least 500 °C, more preferably at least 525 °C. Preferably the coiling temperature is at most 650°C, more preferably at most 625 °C. By decreasing the allowable range of coiling temperatures the homogeneity of the microstructure improves.

The hot-rolled material is subsequently pickled and cold-rolled, preferably with a reduction of at least 40 % and/or at most 80 %. The cold-rolled material is then annealed in a continuous annealing furnace. This is essential, because the batch annealed process does not result in the desired properties of the annealed strip, it is economically very unattractive, and as the heating and cooling during annealing determines the final microstructure and properties it results in an inhomogeneous product as a result of the very slow heating and cooling process which is different for each location in the coil. The time-temperature profile of the heat treatments following the cold rolling are schematically demonstrated in Figure 3. The thickness of the cold rolled-strip depends on the degree of cold rolling reduction and the hot-rolled strip serving as input. The thickness of the cold-rolled strip according to the invention is between 0.3 and 6 mm. Preferably the thickness is at least 0.4 and/or at most 6 mm, more preferably at least 0.6 and/or at most 3.6 mm.

The cold-rolled sheet is annealed at an (δ + γ) intercritical temperature. Because of the difference in recrystallization behaviour between the δ- and the α-phases and the partially reverse transformation of α to γ during intercritical annealing, a microstructure with a bimodal grain size distribution can be obtained during annealing. The recrystallized δ-ferrite has a larger grain size, while the austenite and the α-ferrite have a smaller grain size. The annealing can be performed in a continuous annealing line in a temperature range of 600-900 °C for a duration of between 1 and 600 s.

During an optional initial slow cooling section (see the dashed part (a) in Figure 3), some α-ferrite may form in the austenitic region. This slow cooling causes carbon to be further enriched into the austenite. The stability of the austenite increases as the C content is increased.

The cold-rolling reduction, the annealing time-temperature profile and the subsequent slow cooling process after the annealing are very important for obtaining the final microstructure and the properties of the cold-rolled and annealed strip. The volume fraction and the grain size of various phases as well as the stability of the retained austenite can be adjusted by changing the cold-rolling reduction, the annealing and the subsequent cooling process.

After intercritical annealing and the optional slow cooling, the steel sheet is quenched. Two possible cooling routes are available at this point:
i. direct quenching to ambient temperature
ii. quenching to an austempering temperature, austempering for a certain duration followed by cooling to ambient temperature

The first route involves direct quenching at a cooling rate (CR2) sufficiently high to ambient room temperature. A cooling rate of higher than 10 °C/s is usually sufficient to prevent the decomposition of the austenite for the compositions of the steel according to the invention. A suitable maximum cooling rate is 100 °C/s, preferably at most 75 °C/s, more preferably 50 °C/s. At ambient temperature the final microstructure will consist of δ-ferrite, α-ferrite, martensite and retained austenite.

The second route involves quenching at a cooling rate (CR2) sufficiently high to an temperature between 300 and 500 °C and austempering for a suitable period of 0 to 1200 s. A cooling rate CR2 of higher than 10 °C/s is usually sufficient to prevent the decomposition of the austenite for the compositions of the steel according to the invention. A suitable maximum cooling rate is 100 °C/s, preferably at most 75 °C/s, more preferably 50 °C/s. The austempering temperature must be above the martensite start forming temperature (Ms) and below a bainite start forming temperature (Bs), the exact temperatures of which depend on the steel composition and intercritical annealing temperatures and can be determined e.g. by means of dilatometric experiments. Preferably the austempering annealing takes between 30 and 600 seconds. After the austempering treatment, the steel is cooled to ambient temperature. The cooling rate (CR3) is preferably in the range of 0.01 to 50 °C/s to fit the production line. In the austempering process, the austenite formed during intercritical annealing is decomposed into bainite and retained austenite. Due to the suppression of carbide formation by the high amounts of Al and/or Si during bainitic transformation, the concentration of carbon in the austenite is further increased, so that the stabilization of the retained austenite is further increased. In this case, in addition to the contribution from the ferrite, the retained austenite may be transformed into martensite at room temperature by deformation, so that the ductility is further increased by the TRIP effect.

The average grain size of the δ-ferrite phase is between 5 to 20 µm, preferably at least 7 µm. The average size of the α-ferrite, bainite ferrite, martensite phases and retained austenite is less than 5 µm, preferably less than 3 µm.

The cold-rolled steel may be provided in a known way with a known metallic coating by means of electroplating or hot-dipping, e.g. by hot dip galvanising, preferably wherein the metallic coating is an aluminium based alloy or a zinc-based alloy. Preferably, the galvanizing is carried out in a hot dip galvanizing bath between 400 °C to 500 °C, and then the alloying treatment is carried out at a temperature of 500 °C to 580 °C.

The principles for the alloy design are:
- The steels have complex phase microstructures, including δ-ferrite, α-ferrite, bainitic ferrite, martensite and retained austenite, which have a bimodal grain size distribution.
- The steels contains a quantity of δ-ferrite at all temperatures and at least 10 % in the final microstructure.
- The δ-ferrite has a larger grain size of 5-20 µm. The α-ferrite and remaining phases have a smaller grain size < 5 µm.
- The TRIP effect from the retained austenite transformation contributes to the enhanced formability.
- The δ-ferrite can be retained permanently in the microstructure so that fully martensitic regions are not produced in the heat-affected zone of the spot weld, so the steels may have good weldability.

This microstructure is obtained through composition design and by means of a two-step heat treatment that includes intercritical annealing and quenching (austempering and quenching) for specified compositions. The composition design ensures the presence of the δ-ferrite under equilibrium condition. Al and Si are added to shrink the γ phase field and to obtain the required amount of the δ-ferrite. In the as-cast state, δ-ferrite is generated as dendrites, while pearlitic microstructure is present among the dendritic aims. During reheating and hot-rolling some amount of the δ-ferrite still persists as the reheating and hot-rolling are conducted in the (δ + γ) two phase field. The microstructure after hot-rolling shows a banded structure: layers of the δ-ferrite and austenite, which are elongated along the rolling direction. Depending on the compositions and cooling conditions, the austenite layers may decompose into pearlite, martensite, carbide and retained austenite in the following cooling, as a multi-phase region. During cold-rolling, the δ-phase layers and multiphase layers are further elongated along the rolling direction.

During the intercritical annealing, recrystallization in the δ-phase of the cold-rolled microstructure and reverse transformation in the multiphase regions to austenite occur. Some amount of α-ferrite forms in the original austenite layer during intercritical annealing and during slow cooling in the two-phase area. Bainite, ferrite and martensite form during rapid cooling and austempering and following quenching. Depending on the composition, some residual austenite might be stabilized to room temperature during the final cooling.

In the final microstructure, δ-ferrite is present as layers and has a coarser grain size ranging from 5 to 20 µm, while the α-ferrite and other microstructure in the multiphase regions are much smaller in size, making it a ferrite-(original) austenite duplex steel having a bimodal grain structure, as shown in Figure 4.

According to a third aspect the invention is also embodied in a car, truck or structural or engineering component, such as an automotive chassis component, a component of the body in white, a component of the frame or the subframe, or a component of a structure or engineering project, said component having been produced from the steel sheet according to the invention.

The invention will now be described with reference to the following non-limiting examples.

Steels having compositions shown in Table 1 were cast into ingots of 200 mm x 110 mm x 110 mm in dimensions. The ingots were reheated to 1250 °C and soaked for 1 hour and then rough hot-rolled to 35 mm thickness. The shrinkage and segregation zone from both ends were cut off. The cut blocks were reheated at 1200 °C for 30 min and then hot-rolled to 3 mm thickness in 5 passes. The finish rolling temperature was about 900 °C. It was then cooled in a furnace from 650 °C, after holding at this temperature for 1 h to simulate a coiling procedure. The cooled hot-rolled steel strips were subjected to removal of high-temperature iron oxides from the surface using 10 % HCl solution.

The strip was cold-rolled to produce a 1.2 mm thick steel sheet (60 % reduction). The cold-rolled steel sheet was annealed in a N₂-10 % H₂ atmosphere at a temperature of between 700 and 900 °C for 60 to 180 s, slowly cooled with a cooling rate of 0 or 2 °C/s (CR1) to a temperature between 650 and 800 °C, cooled at a rate of 15 to 30 °C/s (CR2) to a temperature between 480 and 350 °C, maintained at a temperature for a time between 30 and 100 s, and finally cooled to ambient temperature at a rate of 15 to 30 °C/s.

Experiments were also performed in a laboratory scale hot-press forming equipment by Schuler SMG company (SMG press). Steel blanks with dimensions of 200 mm × 110 mm were prepared from a cold-rolled steel sheet. The blanks were subjected to the heat treatment at 800 °C in a box furnace for 300 s and then transferred to the hot-press forming equipment. The press tools were preheated to a temperature of 400 °C. The blanks were transferred to the SMG press in 8 s and press-quenched to 400 °C to form a hot press-formed product. The products were held at 400 °C (austempering) for a time between 30 and 100 s and then cooled to room temperature in air at about 1 °C/s. Tensile specimens were prepared from the flat part of the hot-press-formed product. The tensile properties are similar to the results from the CASIM treatment. So the amount of deformation during hot press forming does not have a significant effect on the final properties.

JIS No. 5 tensile test piece (gauge length = 50 mm) were machined from each annealed sample so that the load axis was parallel to the rolling direction. Room temperature tensile tests were performed in a Schenk TREBEL testing machine following NEN-EN10002-1:2001 standard to determine tensile properties (yield strength YS (MPa), ultimate tensile strength UTS (MPa), total elongation TE (%)). For each condition, three tensile tests were performed and the average values of mechanical properties are reported.

**Table 1. The compositions of the cast steels in wt.%, except N and B in ppm)***

| Steel | C | Mn | Si | Al | Cu | Cr | Ti | N | B | P | S | Sb | Al+Si/3 | ∑** |
|---|---|---|---|---|---|---|---|---|---|---|---|---|---|---|
| A | 0.18 | 3.50 | 0.06 | 4.70 | 0.050 | 0.120 | 0.010 | 50 | - | 0.004 | 0.003 | 0.001 | 4.72 | 2.48 |
| C | 0.13 | 5.80 | 0.25 | 3.20 | 0.010 | 0.020 | 0.020 | 30 | - | 0.005 | 0.002 | 0.002 | 3.28 | 2.82 |
| D | 0.13 | 5.80 | 1.46 | 2.80 | 0.010 | 0.010 | 0.010 | 30 | - | 0.005 | 0.005 | 0.002 | 3.29 | 2.82 |
| E | 0.32 | 5.90 | 0.45 | 4.30 | 0.010 | 0.010 | 0.020 | 20 | - | 0.005 | 0.005 | 0.002 | 4.45 | 3.60 |
| F | 0.35 | 3.50 | 0.06 | 4.40 | 0.010 | 0.010 | 0.040 | 20 | - | 0.005 | 0.004 | 0.001 | 4.42 | 3.15 |
| G | 0.39 | 3.50 | 0.15 | 5.90 | 0.050 | 0.050 | 0.005 | 30 | - | 0.008 | 0.005 | 0.002 | 5.95 | 3.32 |
| H | 0.38 | 1.20 | 0.22 | 3.00 | 0.010 | 0.020 | 0.005 | 30 | - | 0.005 | 0.005 | 0.002 | 3.07 | 2.72 |
| I | 0.38 | 0.60 | 0.21 | 4.10 | 0.020 | 0.020 | 0.005 | 30 | - | 0.006 | 0.004 | 0.003 | 4.17 | 2.57 |
| J | 0.38 | 1.30 | 0.29 | 4.10 | 0.100 | 0.220 | 0.020 | 10 | 10 | 0.010 | 0.001 | 0.005 | 4.20 | 2.76 |

| | | | | | | | | | | | | | | |
|---|---|---|---|---|---|---|---|---|---|---|---|---|---|---|
| * The Ca content in these steels ranges from 0.001 to 0.002, nickel is at impurity level, i.e. below 0.040 wt.%. ** Σ=4C+0.24.Σ(Mn+Cu+Ni)+0.9 | | | | | | | | | | | | | | |

**Table 2. Intercritical annealing, austempering process, tensile properties and volume fraction of the ferritic phase**

| Steel | Annealing | | CR2 | Austempering | | CR3 °C/s | YS MPa | UTS MPa | TE % | δ Vol. % | δ+α Vol. % |
|---|---|---|---|---|---|---|---|---|---|---|---|
| | T (°C) | Time (s) | °C/s | T (°C) | Time (s) | | | | | | |
| A | 800 | 120 | 20 | 400 | 120 | 15 | 489 | 652 | 28.5 | 73 | 79 |
| C1 | 720 | 120 | 20 | RT* | - | - | 814 | 854 | 21.7 | 30 | 68 |
| C2 | 780 | 120 | 20 | RT | - | - | 714 | 994 | 27.5 | 30 | 60 |
| C3 | 840 | 120 | 20 | RT | - | - | 444 | 1161 | 12.4 | 30 | 52 |
| D | 800 | 180 | 20 | 450 | 120 | 15 | 790 | 1038 | 22.8 | 25 | 60 |
| E | 800 | 180 | 20 | 450 | 120 | 15 | 810 | 1245 | 15.6 | 28 | 50 |
| F | 830 | 60 | 10 | 450 | 180 | 15 | 620 | 810 | 28.8 | 46 | 60 |
| G | 830 | 60 | 10 | 400 | 180 | 10 | 677 | 906 | 22 | 35 | 70 |
| H | 850 | 180 | 30 | 450 | 120 | 15 | 545 | 750 | 25.6 | 22 | 50 |
| I | 850 | 180 | 30 | 450 | 120 | 15 | 505 | 661 | 26.4 | 53 | 64 |
| J1 | 850 | 180 | 30 | RT | - | - | 590 | 895 | 22.7 | 50 | 62 |
| J2 | 850 | 180 | 30 | 450 | 60 | 15 | 510 | 800 | 30.2 | 50 | 62 |

| | | | | | | | | | | | |
|---|---|---|---|---|---|---|---|---|---|---|---|
| *RT, room temperature | | | | | | | | | | | |

Figure 1 - This figure shows the various phases occurring in pure iron when slowly cooled from the liquid phase to ambient temperature.

Figure 2 - This shows the phase diagram of steel C, with the (γ + δ) intercritical annealing temperature of 700 to 900 °C marked by the dashed lines.

Figure 3 - This diagram shows the formation of various microstructures during and after the annealing process. RA' denotes a C-enriched RA.

Figure 4 - The SEM micrograph shows a typical example of the bimodal microstructure in the invented steel C after annealing at 780 °C for 120s. The δ-ferrite is revealed as the banded structure with large grain size of average 8 µm, whereas α-ferrite, together with bainite, martensite and retained austenite are shown as blocky islands having a finer grain size less than 3 µm.

## Claims

1. Process for producing a high strength cold-rolled and heat-treated steel strip, sheet, blank or hot-press-formed product having a bimodal microstructure comprising the steps of:
- producing and casting a melt into a slab or cast strip having the following composition;
0.050 - 0.50 wt.% C;
0.500 - 8.00 wt.% Mn;
0.050 - 6.00 wt.% Al_tot;
0 - 0.050 wt.% Sb;
0.0005 - 0.0050 wt.% of Σ (Ca + REM);
5 - 100 ppm N;
0.050 - 2.00 wt.% Si;
0 - 0.020 wt.% S;
0 - 0.050 wt.% P;
0 - 1.00 wt.% Cr;
0 - 2.00 wt.% Ni;
0 - 2.00 wt.% Cu;
0 - 0.50 wt.% Mo;
0 - 0.10 wt.% V;
0 - 50 ppm B;
0 - 0.10 wt.% Ti;
remainder iron and inevitable impurities,
wherein Al + (Si/3) ≥ 4×C+0.24×Σ(Mn+Cu+Ni) + 0.9, and
wherein Σ(Al+Si) is between 0.10 and 6.50 wt.%
- reheating the slab or cast strip to a reheating temperature of between 1100 and 1250 °C;
- hot-rolling the slab or cast strip to a hot-rolled strip wherein the finishing temperature is between 800 and 950 °C;
- cooling and coiling the hot-rolled strip between 680 and 480 °C;
- pickling the hot-rolled strip;
- cold-rolling the pickled hot-rolled strip, preferably with a total cold rolling reduction of between 40 and 80 %;
- optionally producing sheet or blanks from the cold-rolled strip;
- heat treating the steel strip, sheet or blank by intercritically annealing, preferably at a temperature between 600 and 900 °C, for a duration of between 1 and 600 s.
- optionally hot-press-forming the sheet or blank into a hot-press-formed product;
- cooling the annealed steel strip, sheet, blank or hot-press-formed product to an austempering temperature for an austempering treatment between 500 and 300 °C, preferably at most 480 and/or at least 320 °C, at a cooling rate (CR2) which is higher than the critical rate for formation of pearlite, and maintained for a duration of 0 to 1200s for austempering and subsequently cooled to ambient temperature,
so as to obtain an annealed steel strip, sheet, blank or hot-press-formed product with a bimodal grain microstructure consisting of a δ-ferritic phase having an average grain size of between 5 and 20 µm and between 70 and 10 vol.% of a second phase consisting of one or more of α-ferrite with an average grainsize of at most 5 µm, bainite, martensite and/or retained austenite with an average grain size of at most 5 µm, and wherein the final microstructure contains at least 10 vol.% of δ-ferrite, and Σ(δ+α) is between 30 vol.%. and 90 vol.%.

2. Process according to claim 1 wherein the blank undergoes the heat treating in a reheating furnace for a hot-forming press, and wherein the intercritical annealing of the blank takes place before hot-press-forming in the hot-forming press, and wherein the intercritically annealed blank is hot-pressed and cooled at a cooling rate (CR2) which is higher than the critical rate for formation of pearlite to the austempering temperature of between 500 and 300 °C, preferably at most 480 and/or at least 320 °C, in the hot-press and i). held in the hot-press for the duration of the austempering treatment or ii). taken from the hot-press and entered into an austempering furnace, followed by cooling to ambient temperature, preferably at a cooling rate (CR3) of 0.01 °C/s to 50 °C/s.

3. Process according to claim 1 wherein the blank is deformed in a press to form a product and wherein the product subsequently undergoes the heat treating in an annealing furnace wherein the intercritical annealing of the product takes place and wherein
i) the intercritically annealed product is cooled at a cooling rate (CR2) which is higher than the critical rate for formation of pearlite to the austempering temperature of between 500 and 300 °C, preferably at most 480 and/or at least 320 °C, in the annealing furnace and held for the duration of the austempering treatment for 0 to 1200 s, followed by cooling to ambient temperature, preferably at a cooling rate (CR3) of 0.01 °C/s to 50 °C/s, or
ii) wherein the intercritically annealed product is taken from the annealing furnace and entered into an austempering furnace at the austempering temperature of between 500 and 300 ° C, preferably at most 480 and/or at least 320 °C, followed by cooling to ambient temperature, preferably at a cooling rate (CR3) of 0.01 °C/s to 50 °C/s.

4. Process according to claim 1 wherein the aluminium content of the slab or cast strip is at most 5.50 wt.%.

5. Process according to claim 1 wherein the coiling temperature is at least 475 °C, preferably at least 500 °C and/or at most 650 °C, preferably at most 625 °C.

6. Process according to any one the preceding claims wherein the duration of the intercritical annealing is at least 30 s and/or at most 400 s.

7. Process according to any one the preceding claims wherein the duration of the austempering annealing is at least 30 s and/or at most 600 s.

8. Process according to any one of the preceding claims wherein the austempering temperature is at least 320 °C and preferably at least 350 °C and/or at most 475 °C, and preferably at most 450 °C.

9. Process according to any one of the preceding claims wherein the Sb content is at least 0.0005 wt.%.

10. Process according to any one of the preceding claims wherein Σ(Mn+Cu+Ni) is between 0.50 and 8.00 wt.%.

11. Process according to any one of the preceding claims wherein the total cold-rolling reduction is between 40 and 80 %, and/or wherein the strip, sheet or blank is provided with a metallic coating by means of plating or hot-dipping, preferably wherein the metallic coating is an aluminium based alloy or a zinc based alloy.

12. High strength cold-rolled and heat-treated steel strip, sheet, blank or hot-press-formed product having a bimodal microstructure having the following composition;
0.050 - 0.50 wt.% C;
0.500 - 8.00 wt.% Mn;
0.050 - 6.00 wt.% Al_tot;
0 - 0.050 wt.% Sb;
0.0005 - 0.0050 wt.% of Σ (Ca + REM);
5 - 100 ppm N;
0.050 - 2.00 wt.% Si;
0 - 0.020 wt.% S;
0 - 0.050 wt.% P;
0 - 1.00 wt.% Cr;
0 - 2.00 wt.% Ni;
0 - 2.00 wt.% Cu;
0 - 0.50 wt.% Mo;
0 - 0.10 wt.% V;
0 - 50 ppm B;
0 - 0.10 wt.% Ti;
wherein Al + (Si/3) ≥ 4×C+0.24×Σ(Mn+Cu+Ni) + 0.9, and
wherein Σ(Al+Si) is between 0.10 and 6.50 wt.%
remainder iron and inevitable impurities, remainder iron and inevitable impurities,
- wherein the heat treated steel strip, sheet, blank or hot-press-formed product has a bimodal grain microstructure consisting of δ-ferrite and α-ferrite, wherein the δ-ferrite has an average grain size of between 5 and 20 µm, wherein the α-ferrite has an average grain size of at most 5 µm and between 70 and 10 vol.% of a second phase consisting of one or more of bainite, martensite and/or retained austenite with an average grain size of at most 5 µm, and wherein the final microstructure contains at least 10 % of δ-ferrite, and Σ(δ+α) is between 30 vol.%. and 90 vol.%, said high strength cold-rolled and heat-treated steel strip, sheet, blank or hot-press formed product being obtainable by the process according to any one of claims 1 to 11.

13. High strength cold-rolled and heat-treated steel strip, sheet, blank or hot-press-formed product having a bimodal microstructure consisting of δ-ferrite and α-ferrite, according to claim 12 wherein the δ-ferrite has an average grain size of between 5 and 20 µm, wherein the α-ferrite has an average grain size of at most 3 µm and a second phase consisting of one or more of bainite, martensite and/or retained austenite with an average grain size of at most 3 µm.

14. High strength cold-rolled and heat-treated steel strip, sheet, blank or hot-press-formed product according to claim 12 or 13 wherein the aluminium content of the slab or cast strip is at most 5.50 wt.%.

15. High strength cold-rolled and heat-treated steel strip, sheet, blank or hot-press-formed product according to claim 12 or 13 wherein the steel is coated with a metallic coating by means of plating or hot-dipping, preferably wherein the metallic coating is an aluminium based alloy or a zinc based alloy.

16. Component, e.g. a car or truck component, such as an automotive chassis component, a component of the body in white, a component of the frame or the subframe, or a component of a structure or engineering project, said component being a product according to claim 12, wherein the component has a bimodal grain microstructure consisting of δ-ferrite and α-ferrite, wherein the δ-ferrite has an average grain size of between 5 and 20 µm, wherein the α-ferrite has an average grain size at most 3 µm and a second phase consisting of one or more of bainite, martensite and/or retained austenite with an average grain size of at most 5 µm.

17. Component according to claim 16 wherein the component has a bimodal grain microstructure consisting of δ-ferrite and α-ferrite, wherein the δ-ferrite has an average grain size of between 5 and 20 µm, wherein the α-ferrite has an average grain size of at most 3 µm and a second phase consisting of one or more of bainite, martensite and/or retained austenite with an average grain size of at most 3 µm.

## Patentansprüche

1. Verfahren zum Herstellen eines Bandes, Blechs, Rohlings oder eines warmpressgeformten Produktes aus hochfestem kaltgewalztem und wärmebehandeltem Stahl mit einer bimodalen Mikrostruktur, die folgenden Schritte umfassend:
- Herstellen und Gießen einer Schmelze in eine Bramme oder ein Gussband, die die folgende Zusammensetzung aufweist;
0,050 - 0,50 Gew.-% C;
0,500 - 8,00 Gew.-% Mn;
0,050 - 6,00 Gew.-% Al_tot;
0 - 0,050 Gew.-% Sb;
0,0005 - 0,0050 Gew.-% Σ (Ca + REM);
5 - 100 ppm N;
0,050 - 2,00 Gew.-% Si;
0 - 0,020 Gew.-% S;
0 - 0,050 Gew.-% P;
0 - 1,00 Gew.-% Cr;
0 - 2,00 Gew.-% Ni;
0 - 2,00 Gew.-% Cu;
0 - 0,50 Gew.-% Mo;
0 - 0,10 Gew.-% V;
0 - 50 ppm B;
0 - 0,10 Gew.-% Ti;
Rest aus Eisen und unvermeidbaren Verunreinigungen,
wobei Al + (Si/3) ≥ 4×C + 0,24×∑(Mn+Cu+Ni) + 0,9 und
wobei Σ(Al+Si) zwischen 0,10 und 6,50 Gew.-% liegt,
- Wiedererwärmen der Bramme oder des Gussbandes auf eine Wiedererwärmungstemperatur zwischen 1100 und 1250 °C;
- Warmwalzen der Bramme oder des Gussbandes zu einem warmgewalzten Band, wobei die Endtemperatur 800 bis 950 °C beträgt;
- Kühlen und Aufwickeln des warmgewalzten Bandes zwischen 680 und 480 °C;
- Beizen des warmgewalzten Bandes;
- Kaltwalzen des gebeizten warmgewalzten Bandes, bevorzugt mit einer Gesamtkaltwalzreduktion zwischen 40 und 80 %;
- optional Herstellen von Blechen oder Rohlingen aus dem kaltgewalzten Band;
- Wärmebehandeln des Bandes, Blechs oder Rohlings aus Stahl durch interkritisches Glühen, bevorzugt bei einer Temperatur zwischen 600 und 900 °C, über eine Dauer zwischen 1 und 600 s,
- optional Warmpressformen des Blechs oder des Rohlings zu einem warmpressgeformten Produkt;
- Kühlen des geglühten Bandes, Blechs, Rohlings oder warmpressgeformten Produkts aus Stahl auf eine Zwischenstufenvergütungstemperatur für eine Zwischenstufenvergütungsbehandlung zwischen 500 und 300 °C, bevorzugt höchstens 480 und/oder mindestens 320 °C, bei einer Kühlrate (CR2), die höher als die kritische Rate für eine Ausbildung von Perlit ist, und die über eine Dauer von 0 bis 1200 s zum Zwischenstufenvergüten aufrechterhalten und anschließend auf Umgebungstemperatur gekühlt wird,
um ein geglühtes Band, Blech, einen Rohling oder ein warmpressgeformtes Produkt aus Stahl mit einer bimodalen Kornmikrostruktur zu erhalten, die aus einer δ-ferritischen Phase mit einer durchschnittlichen Korngröße zwischen 5 und 20 µm und zwischen 70 und 10 Vol.-% einer zweiten Phase besteht, die aus einem oder mehreren von α-Ferrit mit einer durchschnittlichen Korngröße von höchstens 5 µm, Bainit, Martensit und/oder Restaustenit mit einer durchschnittlichen Korngröße von höchstens 5 µm besteht, und wobei die finale Mikrostruktur mindestens 10 Vol.-% δ-Ferrit enthält und Σ(δ+α) zwischen 30 Vol.-% und 90 Vol.-% liegt.

2. Verfahren nach Anspruch 1, wobei der Rohling der Wärmebehandlung in einem Wiedererwärmungsofen für eine Warmformpresse unterzogen wird und wobei das interkritische Glühen des Rohlings vor dem Warmpressformen in der Warmformpresse stattfindet und wobei der interkritisch geglühte Rohling warmgepresst und mit einer Kühlrate (CR2), die höher als die kritische Rate für eine Ausbildung von Perlit ist, auf die Zwischenstufenvergütungstemperatur zwischen 500 und 300 °C, vorzugsweise höchstens 480 und/oder mindestens 320 °C, in der Warmpresse gekühlt wird und i). für die Dauer der Zwischenstufenvergütungsbehandlung in der Warmpresse gehalten wird oder ii). aus der Warmpresse entnommen und in einen Zwischenstufenvergütungsofen eingeleitet wird, gefolgt von Abkühlen auf Umgebungstemperatur, vorzugsweise mit einer Kühlrate (CR3) von 0,01 °C/s bis 50 °C/s.

3. Verfahren nach Anspruch 1, wobei der Rohling in einer Presse umgeformt wird, um ein Produkt zu formen, und wobei das Produkt anschließend der Wärmebehandlung in einem Glühofen unterzogen wird, wobei das interkritische Glühen des Produkts stattfindet, und wobei
i) das interkritisch geglühte Produkt mit einer Kühlrate (CR2), die höher als die kritische Rate für eine Ausbildung von Perlit ist, auf die Zwischenstufenvergütungstemperatur zwischen 500 und 300 °C, vorzugsweise höchstens 480 und/oder mindestens 320 °C, in dem Glühofen gekühlt und während der Dauer der Zwischenstufenvergütungsbehandlung für 0 bis 1200 s gehalten wird, gefolgt von Abkühlen auf Umgebungstemperatur, vorzugsweise mit einer Kühlrate (CR3) von 0,01 °C/s bis 50 °C/s, oder
ii) wobei das interkritisch geglühte Produkt aus dem Glühofen entnommen und bei der Zwischenstufenvergütungstemperatur zwischen 500 und 300 °C, vorzugsweise höchstens 480 und/oder mindestens 320 °C, in einen Zwischenstufenvergütungsofen eingeleitet wird, gefolgt von Abkühlen auf Umgebungstemperatur, vorzugsweise mit einer Kühlrate (CR3) von 0,01 °C/s bis 50 °C/s.

4. Verfahren nach Anspruch 1, wobei der Aluminiumgehalt der Bramme oder des Gussbandes höchstens 5,50 Gew.-% beträgt.

5. Verfahren nach Anspruch 1, wobei die Aufwickeltemperatur mindestens 475 °C, vorzugsweise mindestens 500 °C und/oder höchstens 650 °C, vorzugsweise höchstens 625 °C beträgt.

6. Verfahren nach einem der vorhergehenden Ansprüche, wobei die Dauer des interkritischen Glühens mindestens 30 s und/oder höchstens 400 s beträgt.

7. Verfahren nach einem der vorhergehenden Ansprüche, wobei die Dauer des Zwischenstufenvergütungsglühens mindestens 30 s und/oder höchstens 600 s beträgt.

8. Verfahren nach einem der vorhergehenden Ansprüche, wobei die Zwischenstufenvergütungstemperatur mindestens 320 °C und vorzugsweise mindestens 350 °C und/oder höchstens 475 °C und vorzugsweise höchstens 450 °C beträgt.

9. Verfahren nach einem der vorhergehenden Ansprüche, wobei der Sb-Gehalt mindestens 0,0005 Gew.-% beträgt.

10. Verfahren nach einem der vorhergehenden Ansprüche, wobei Σ(Mn+Cu+Ni) zwischen 0,50 und 8,00 Gew.-% beträgt.

11. Verfahren nach einem der vorhergehenden Ansprüche, wobei die gesamte Kaltwalzreduktion zwischen 40 und 80 % liegt und/oder wobei das Band, Blech oder der Rohling mit einer metallischen Beschichtung mittels Galvanisieren oder Schmelztauchen versehen wird, wobei die metallische Beschichtung vorzugsweise eine Legierung auf Aluminiumbasis oder eine Legierung auf Zinkbasis ist.

12. Band, Blech, Rohling oder warmpressgeformtes Produkt aus hochfestem kaltgewalztem und wärmebehandeltem Stahl mit einer bimodalen Mikrostruktur, die folgende Zusammensetzung aufweisend;
0,050 - 0,50 Gew.-% C;
0,500 - 8,00 Gew.-% Mn;
0,050 - 6,00 Gew.-% Al_tot;
0 - 0,050 Gew.-% Sb;
0,0005 - 0,0050 Gew.-% Σ (Ca + REM);
5 - 100 ppm N;
0,050 - 2,00 Gew.-% Si;
0 - 0,020 Gew.-% S;
0 - 0,050 Gew.-% P;
0 - 1,00 Gew.-% Cr;
0 - 2,00 Gew.-% Ni;
0 - 2,00 Gew.-% Cu;
0 - 0,50 Gew.-% Mo;
0 - 0,10 Gew.-% V;
0 - 50 ppm B;
0 - 0,10 Gew.-% Ti;
wobei Al + (Si/3) ≥ 4×C + 0,24×∑(Mn+Cu+Ni) + 0,9 und
wobei Σ(Al+Si) zwischen 0,10 und 6,50 Gew.-% liegt,
Rest aus Eisen und unvermeidbaren Verunreinigungen,
- wobei das Band, Blech, der Rohling oder das warmpressgeformte Produkt aus wärmebehandeltem Stahl eine bimodale Kornmikrostruktur aufweist, die aus δ-Ferrit und α-Ferrit besteht, wobei der δ-Ferrit eine durchschnittliche Korngröße zwischen 5 und 20 µm aufweist, wobei der α-Ferrit eine durchschnittliche Korngröße von höchstens 5 µm aufweist, und aus zwischen 70 und 10 Vol.-% einer zweiten Phase, die aus einem oder mehreren von Bainit, Martensit und/oder Restaustenit mit einer durchschnittlichen Korngröße von höchstens 5 µm besteht, und wobei die finale Mikrostruktur mindestens 10 % δ-Ferrit enthält und ∑(δ+α) zwischen 30 Vol.-% und 90 Vol.-% liegt, wobei das Band, Blech, der Rohling oder das warmpressgeformte Produkt aus hochfestem kaltgewalztem und wärmebehandeltem Stahl durch das Verfahren nach einem der Ansprüche 1 bis 11 erlangbar ist.

13. Band, Blech, Rohling oder warmpressgeformtes Produkt aus hochfestem kaltgewalztem und wärmebehandeltem Stahl mit einer bimodalen Mikrostruktur, die aus δ-Ferrit und α-Ferrit besteht, nach Anspruch 12, wobei der δ-Ferrit eine durchschnittliche Korngröße zwischen 5 und 20 µm aufweist, wobei der α-Ferrit eine durchschnittliche Korngröße von höchstens 3 µm aufweist, und aus einer zweiten Phase, die aus einem oder mehreren von Bainit, Martensit und/oder Restaustenit mit einer durchschnittlichen Korngröße von höchstens 3 µm besteht.

14. Band, Blech, Rohling oder warmpressgeformtes Produkt aus hochfestem kaltgewalztem und wärmebehandeltem Stahl nach Anspruch 12 oder 13, wobei der Aluminiumgehalt der Bramme oder des Gussbandes höchstens 5,50 Gew.-% beträgt.

15. Band, Blech, Rohling oder warmpressgeformtes Produkt aus hochfestem kaltgewalztem und wärmebehandeltem Stahl nach Anspruch 12 oder 13, wobei der Stahl mit einer metallischen Beschichtung mittels Galvanisieren oder Schmelztauchen beschichtet ist, wobei die metallische Beschichtung vorzugsweise eine Legierung auf Aluminiumbasis oder eine Legierung auf Zinkbasis ist.

16. Komponente, z. B. eine PKW- oder LKW-Komponente, wie eine Automobilfahrgestellkomponente, eine Komponente der Rohkarosserie, eine Komponente des Rahmens oder des Hilfsrahmens oder eine Komponente einer Struktur oder eines technischen Projekts, wobei die Komponente ein Produkt gemäß Anspruch 12 ist, wobei die Komponente eine bimodale Kornmikrostruktur aufweist, die aus δ-Ferrit und α-Ferrit besteht, wobei der δ-Ferrit eine durchschnittliche Korngröße zwischen 5 und 20 µm aufweist, wobei der α-Ferrit eine durchschnittliche Korngröße von höchstens 3 µm aufweist, und aus einer zweiten Phase , die aus einem oder mehreren von Bainit, Martensit und/oder Restaustenit mit einer durchschnittlichen Korngröße von höchstens 5 µm besteht.

17. Komponente nach Anspruch 16, wobei die Komponente eine bimodale Kornmikrostruktur aufweist, die aus δ-Ferrit und α-Ferrit besteht, wobei der δ-Ferrit eine durchschnittliche Korngröße zwischen 5 und 20 µm aufweist, wobei der α-Ferrit eine durchschnittliche Korngröße von höchstens 3 µm aufweist, und aus einer zweiten Phase, die aus einem oder mehreren von Bainit, Martensit und/oder Restaustenit mit einer durchschnittlichen Korngröße von höchstens 3 µm besteht.

## Revendications

1. Procédé destiné à produire une bande, une feuille, un flan ou un produit formé par pressage à chaud, en acier à haute résistance laminé à froid et traité thermiquement, présentant une microstructure bimodale comprenant les étapes suivantes :
- la production et la coulée d'une masse fondue en une brame ou une bande coulée présentant la composition suivante ;
0,050 à 0,50 % en poids de C ;
0,500 à 8,00 % en poids de Mn ;
0,050 à 6,00 % en poids d'Al_tot ;
0 à 0,050 % en poids de Sb ;
0,0005 à 0,0050 % en poids de Σ (Ca + REM) ;
5 à 100 ppm de N ;
0,050 à 2,00 % en poids de Si ;
0 à 0,020 % en poids de S ;
0 à 0,050% en poids de P ;
0 à 1,00 % en poids de Cr ;
0 à 2,00 % en poids de Ni ;
0 à 2,00 % en poids de Cu ;
0 à 0,50 % en poids de Mo ;
0 à 0,10% en poids de V ;
0 à 50 ppm de B ;
0 à 0,10 % en poids de Ti ;
le reste étant du fer et des impuretés inévitables ;
dans lequel Al + (Si/3) ≥ 4×C+0,24×Σ(Mn+Cu+Ni) + 0,9 et
dans lequel Σ(Al+Si) est comprise entre 0,10 et 6,50 % en poids
- le réchauffage de la brame ou de la bande coulée à une température de réchauffage comprise entre 1 100 et 1 250 °C ;
- le laminage à chaud de la brame ou de la bande coulée en une bande laminée à chaud dans lequel la température de finition est comprise entre 800 et 950 °C ;
- le refroidissement et l'enroulement de la bande laminée à chaud entre 680 et 480 °C ;
- le décapage de la bande laminée à chaud ;
- le laminage à froid de la bande laminée à chaud décapée, de préférence avec une réduction totale par laminage à froid comprise entre 40 et 80 % ;
- éventuellement, la production d'une feuille ou de flans à partir de la bande laminée à froid ;
- le traitement thermique de la bande, de la feuille ou du flan d'acier par recuit intercritique, de préférence à une température comprise entre 600 et 900 °C, pendant une durée comprise entre 1 et 600 s,
- éventuellement, le formage par pressage à chaud de la feuille ou du flan en un produit formé par pressage à chaud ;
- le refroidissement de la bande d'acier, de la feuille, du flan ou du produit formé par pressage à chaud recuit à une température de trempe pour un traitement de trempe compris entre 500 et 300 °C, de préférence au plus 480 et/ou au moins 320 °C, à une vitesse de refroidissement (CR2) supérieure à la vitesse critique de formation de perlite, et maintenu pendant une durée de 0 à 1200 s pour la trempe et ensuite refroidi à température ambiante,
de manière à obtenir une bande, une feuille, un flan ou un produit formé par pressage à chaud en acier recuit présentant une microstructure bimodale à grains constituée par une phase δ-ferritique présentant une taille moyenne de grain comprise entre 5 et 20 µm et entre 70 et 10 % en volume d'une seconde phase constituée d'un ou de plusieurs éléments parmi de l'α-ferrite présentant une taille moyenne d'au plus 5 µm, de la bainite, de la martensite et/ou de l'austénite retenue présentant une taille moyenne de grain d'au plus 5 µm, et dans lequel la microstructure finale contient au moins 10 % en volume de δ-ferrite, et Σ(δ+α) est comprise entre 30 % en volume et 90 % en volume.

2. Procédé selon la revendication 1, dans lequel le flan subit le traitement thermique dans un four de réchauffage pour une presse de formage à chaud, et dans lequel le recuit intercritique du flan a lieu avant le formage par pressage à chaud dans la presse de formage à chaud, et dans lequel le flan recuit intercritiquement est pressé à chaud et refroidi à une vitesse de refroidissement (CR2) supérieure à la vitesse critique pour la formation de perlite à la température de trempe comprise entre 500 et 300 °C, de préférence au plus 480 et/ou au moins 320 °C, dans la presse à chaud et i) maintenu dans la presse à chaud pendant la durée du traitement de trempe ou ii). extrait de la presse à chaud et introduit dans un four de trempe, suivi d'un refroidissement à température ambiante, de préférence à une vitesse de refroidissement (CR3) de 0,01 °C/s à 50 °C/s.

3. Procédé selon la revendication 1, dans lequel le flan est déformé dans une presse pour former un produit et dans lequel le produit subit ensuite le traitement thermique dans un four de recuit dans lequel le recuit intercritique du produit a lieu et dans lequel
i) le produit recuit intercritiquement est refroidi à une vitesse de refroidissement (CR2) supérieure à la vitesse critique de formation de perlite à la température de trempe comprise entre 500 et 300 °C, de préférence au plus 480 et/ou au moins 320 °C, et maintenu pendant la durée du traitement de trempe pendant 0 à 1200 s, suivi d'un refroidissement à température ambiante, de préférence à une vitesse de refroidissement (CR3) de 0,01 °C/s à 50 °C/s, ou
ii) dans lequel le produit recuit intercritiquement est extrait du four de recuit et introduit dans un four de trempe à la température de trempe comprise entre 500 et 300 °C, de préférence au plus 480 et/ou au moins 320 °C, suivi d'un refroidissement aux températures ambiantes, de préférence à une vitesse de refroidissement (CR3) de 0,01 °C/s à 50 °C/s.

4. Procédé selon la revendication 1, dans lequel la teneur en aluminium de la brame ou de la bande coulée est d'au plus 5,50 % en poids.

5. Procédé selon la revendication 1, dans lequel la température d'enroulement est d'au moins 475 °C, de préférence d'au moins 500 °C et/ou d'au plus 650 °C, de préférence d'au plus 625 °C.

6. Procédé selon l'une quelconque des revendications précédentes, dans lequel la durée du recuit intercritique est d'au moins 30 s et/ou d'au plus 400 s.

7. Procédé selon l'une quelconque des revendications précédentes, dans lequel la durée du recuit de trempe est d'au moins 30 s et/ou d'au plus 600 s.

8. Procédé selon l'une quelconque des revendications précédentes, dans lequel la température de trempe est d'au moins 320 °C, de préférence d'au moins 350 °C et/ou d'au plus 475 °C et de préférence d'au plus 450 °C.

9. Procédé selon l'une quelconque des revendications précédentes, dans lequel la teneur en Sb est d'au moins 0,0005 % en poids.

10. Procédé selon l'une quelconque des revendications précédentes, dans lequel Σ(Mn+Cu+Ni) est comprise entre 0,50 et 8,00 % en poids.

11. Procédé selon l'une quelconque des revendications précédentes, dans lequel la réduction totale par laminage à froid est comprise entre 40 et 80 %, et/ou dans lequel la bande, la feuille ou le flan est pourvu d'un revêtement métallique par placage ou trempage à chaud, de préférence dans lequel le revêtement métallique est un alliage à base d'aluminium ou un alliage à base de zinc.

12. Bande, feuille, flan ou produit formé par pressage à chaud, en acier à haute résistance laminé à froid et traité thermiquement présentant une microstructure bimodale présentant la composition suivante :
0,050 à 0,50 % en poids de C ;
0,500 à 8,00 % en poids de Mn ;
0,050 à 6,00 % en poids d'Al_tot ;
0 à 0,050 % en poids de Sb ;
0,0005 à 0,0050 % en poids de Σ (Ca + REM) ;
5 à 100 ppm de N ;
0,050 à 2,00 % en poids de Si ;
0 à 0,020 % en poids de S ;
0 à 0,050% en poids de P ;
0 à 1,00 % en poids de Cr ;
0 à 2,00 % en poids de Ni ;
0 à 2,00 % en poids de Cu ;
0 à 0,50 % en poids de Mo ;
0 à 0,10% en poids de V ;
0 à 50 ppm de B ;
0 à 0,10 % en poids de Ti ;
dans lequel Al + (Si/3) ≥ 4×C+0,24×Σ(Mn+Cu+Ni) + 0,9 et
dans lequel Σ(Al+Si) est comprise entre 0,10 et 6,50 % en poids
le reste étant du fer et des impuretés inévitables,
- dans lequel la bande, la feuille, le flan ou le produit formé par pressage à chaud en acier traité thermiquement présente une microstructure bimodale à grains constituée de δ-ferrite et d'α-ferrite, dans lequel la δ-ferrite présente une taille moyenne de grain comprise entre 5 et 20 µm, dans lequel l'α-ferrite présente une taille moyenne de grain d'au plus 5 µm et entre 70 et 10 % en volume d'une seconde phase constituée d'un ou plusieurs éléments parmi de la bainite, de la martensite et/ou de l'austénite retenue présentant une taille moyenne de grain d'au plus 5 µm, et dans lequel la microstructure finale contient au moins 10 % de δ-ferrite, et Σ(δ+α) est comprise entre 30 % en volume et 90 % en volume, ladite bande, ladite feuille, ledit flan ou ledit produit formé par pressage à chaud, en acier à haute résistance laminé à froid et traité thermiquement pouvant être obtenu par le procédé selon l'une quelconque des revendications 1 à 11.

13. Bande, feuille, flan ou produit formé par pressage à chaud en acier laminé à froid et traité thermiquement à haute résistance présentant une microstructure bimodale constituée de δ-ferrite et d'α-ferrite, selon la revendication 12, dans lequel la δ-ferrite présente une taille moyenne de grain comprise entre 5 et 20 µm, dans lequel l'α-ferrite présente une taille moyenne de grain d'au plus 3 µm et une seconde phase constituée d'un ou de plusieurs éléments parmi de la bainite, de la martensite et/ou de l'austénite retenue présentant une taille moyenne de grain d'au plus 3 µm.

14. Bande, feuille, flan ou produit formé par pressage à chaud, en acier à haute résistance laminé à froid et traité thermiquement selon la revendication 12 ou 13, dans lequel la teneur en aluminium de la brame ou de la bande coulée est d'au plus 5,50 % en poids.

15. Bande, feuille, flan ou produit formé par pressage à chaud, en acier à haute résistance laminé à froid et traité thermiquement selon la revendication 12 ou 13, dans lequel l'acier est revêtu d'un revêtement métallique au moyen d'un placage ou d'un trempage à chaud, de préférence dans lequel le revêtement métallique est un alliage à base d'aluminium ou un alliage à base de zinc.

16. Composant, par exemple un composant de voiture ou de camion, tel qu'un composant de châssis de véhicule, un composant de la carrosserie en blanc, un composant du cadre ou du sous-châssis, ou un composant d'une structure ou d'un projet d'ingénierie, ledit composant étant un produit selon la revendication 12,
dans lequel le composant présente une microstructure de grain bimodal constituée de δ-ferrite et d'α-ferrite, dans lequel la δ-ferrite présente une taille moyenne de grain comprise entre 5 et 20 µm, dans lequel l'α-ferrite présente une taille moyenne de grain d'au plus 3 µm et une seconde phase constituée d'un ou de plusieurs éléments parmi de la bainite, de la martensite et/ou de l'austénite retenue présentant une taille moyenne de grain d'au plus 5 µm.

17. Composant selon la revendication 16, dans lequel le composant présente une microstructure de grain bimodal constituée de δ-ferrite et d'α-ferrite, dans lequel la δ-ferrite présente une taille moyenne de grain comprise entre 5 et 20 µm, dans lequel l'α-ferrite présente une taille moyenne de grain d'au plus 3 µm et une seconde phase constituée d'un ou de plusieurs éléments parmi de la bainite, de la martensite et/ou de l'austénite retenue présentant une taille moyenne de grain d'au plus 3 µm.
